

# UNITED STATES PATENT OFFICE.

LAURENCE G. WESSON, OF CLEVELAND, AND ZAY JEFFRIES, OF EAST CLEVELAND,  
OHIO

## STROP-DRESSING.

1,327,648.

Specification of Letters Patent.

Patented Jan. 13, 1920.

No Drawing.

Application filed December 1, 1916. Serial No. 134,380.

*To all whom it may concern:*

Be it known that we, LAURENCE G. WESSON, residing in Cleveland, in the county of Cuyahoga, in the State of Ohio, at 1719 5 East 116th Place, and ZAY JEFFRIES, residing in East Cleveland, in the county of Cuyahoga, in the State of Ohio, at 328 Carlton road, both citizens of the United States, have invented a new and useful Strop-Dress-10 ing.

The invention relates to a composition including as a constituent an abrasive substance adapted to render a strop or other suitable surface, to which it is applied, an 15 effective sharpening agent for razors, surgical instruments, and the like.

The general objects of our invention are: (1) to provide a strop dressing with an abrasive adapted to give an extremely fine 20 cutting edge to the razor or instrument to be sharpened; (2) to provide a dressing in which the vehicle for the abrasive substance is of such a nature that the dressing can readily be applied to a strop and readily 25 renewed from time to time so that the strop can easily be kept in an effective condition; and (3) to provide a dressing for razor strops which will not injure either the strop or the steel of the razor and which will be 30 harmless if inadvertently taken into the mouth or applied to the skin.

Our invention has other objects but they are largely ancillary to the foregoing and will be made clear in the following description setting forth in detail the preferred 35 constituent materials for the composition, the preferred method of combining the said materials and the preferred manner of using the dressing.

From our experience with various materials, we have found that an abrasive in the 40 form of superfine levigated alumina is especially adapted to our purposes and we use it in carrying out our invention. The 45 levigated alumina available on the market can be used with a fair degree of satisfaction. It is not of uniform fineness, however, and if it is permitted to settle in water, or other suitable liquid, the coarser particles will sink to the bottom first, the rate 50 of settling being proportional to the size of the particles. That portion of the powder which settles out during the first six or eight hours, say, is relatively coarse, while

that which remains in suspension after more 55 prolonged sedimentation, say twenty-four hours, is found to be exceedingly fine. Thus by subjecting the commercial levigated alumina to such prolonged sedimentation and separating the material which remains in 60 suspension, we secure a superfine product which is peculiarly adapted to the carrying out of our invention both because it is well suited for the production of an extremely 65 fine cutting edge and also because it is adapted for the production of a relatively permanent emulsion when combined with materials which we employ as a vehicle for it.

In order that the dressing may readily be 70 applied and renewed on the strop, we utilize a vehicle for the abrasive which is readily soluble in water and we have found that a suitable mixture of soap and water is most effective for this purpose. We preferably 75 use soap in powdered form.

We also prefer to provide a vehicle for 80 the abrasive that is either inherently antiseptic or capable of being rendered so, and this is readily accomplished with the soap and water vehicle by the addition of a suitable amount of an antiseptic in liquid form such as phenol or thymol.

In the preparation of the dressing the 85 preferable procedure is as follows. The powdered soap and the levigated alumina, are first intimately mixed in the desired proportions. Then successive portions of water are added until the desired consistency 90 is secured, the whole being vigorously mixed as the water is added. The antiseptic, when used, may conveniently be added to the water and is then distributed by the mixing operation. If desired, an agreeable odor may 95 be imparted to the dressing by the addition of any substance suitable for the purpose.

In so far as some aspects of our invention 100 are concerned the essential constituents may be used in any proportions which will give a dressing capable of use for the purposes in question; but in order to secure a dressing that can be conveniently packed for distribution and use and that can conveniently, easily and quickly be applied to a strop, we greatly prefer to combine the constituents in proportions such that the product has the 105 consistency of a cream or paste.

This end is more or less fully attained if the proportions by weight of the several es-

ential constituents are kept within the following limits:

5      Levigated alumina 30% to 50%,  
          Powdered soap 10% to 25%,  
          Water 30% to 55%.

The proper consistency may be considered as the one which a maximum amount of the levigated alumina is incorporated into a 10 paste having the desired properties as described above. If too much water is added, the abrasive has a tendency to settle and thus destroy the uniform consistency and character of the paste. In practice we prefer the following proportions by weight:

Levigated alumina 47%,  
Powdered soap 20%,  
Water 33%.

20     When the preferred constituents are properly combined in the manner above described and in the proportions last referred to, a comparatively permanent emulsion having the consistency of a cream or paste is produced. As we have intimated, the superfine levigated alumina and the vehicle employed seem especially adapted to produce such an emulsion-like mixture in which the abrasive is held for indefinite periods uniformly distributed in suspension in the 25 cream-like body.

Obviously a composition having the consistency last referred to is admirably adapted to be packed in and dispensed from collapsible metal tubes, and we prefer to use containers of this character because of their great convenience.

In the use of our improved dressing a small amount, say twice the volume of a pea, 40 is expelled from the tube or other container on the strop. The user can then readily spread the dressing evenly over the surfaces of the strop either with his wetted fingers or a moist cloth. Then, either immediately 45 or after waiting a few minutes until the water added to the paste in order to facilitate spreading has evaporated, the stropping of the razor can be proceeded with in the ordinary manner. In the case of a very 50 dull blade a considerable number of strokes may be required to secure a thoroughly sharp edge, but a razor which is in fairly good condition needs only a few strokes to sharpen it perfectly. It will be understood that our 55 dressing is applied to but one surface of the strop and that the sharpening operation can if desired be completed on another, finishing surface in the usual manner.

When our improved dressing has been applied to a strop in the manner described, 60 the strop can be used effectively for ten or twelve days and then, if the best results are to be secured, the surface of the strop should be cleaned and renewed with a fresh application of the dressing. As far as we are

aware, the abrasive dressings which have heretofore been proposed have been exceedingly unsatisfactory in this connection. In fact, we are of the opinion that the abrasive dressings heretofore proposed have been unsuccessful in practice because of the difficulty in some cases, of applying the dressing to the strop, and in other cases, of removing the dressing and securing a clean strop surface prior to a fresh application of the dressing. In the case of our improved dressing these difficulties have been entirely overcome by the provision of a vehicle for the abrasive in the form of a permanent emulsion which is soluble in water. By 70 reason of its consistency and solubility the fresh dressing can be easily applied and the old dressing can be removed very quickly and with the greatest ease by means of a wet sponge, cloth or the like, and thereupon 75 a fresh dressing can be applied in the manner above described. A strop which is treated in the manner indicated may, by periodically renewing our improved dressing, be kept indefinitely in highly effective 80 condition, no difficulty being experienced from the accumulation of a gummy coating on the strop which is characteristic of dressing employing oily or greasy substances 85 as a vehicle for the abrasive.

It is clear that we have not only provided a dressing adapted to render the strop an effective sharpening agent but also that none of the constituent materials of the dressing are of a nature to injure either 90 the strop or the steel of the razor or instrument blade. It will also be seen that the dressing is harmless if the dressing should be mistaken for tooth paste, cold cream, or the like, and inadvertently taken 95 into the mouth or applied to the skin. Furthermore, the dressing is readily washed from the skin, as when the user spreads it on a strop with his fingers, and its use is both convenient and pleasant in this respect.

We are aware that preparations comprising a mixture of soap and powdered abrasive have heretofore been proposed, but we do not know of any proposal to so use levigated or finely divided alumina. Nor 105 do we know of any proposal to use a preparation of finely divided abrasive, soap and water in proportions to form a relatively permanent emulsion having the consistency of a cream or paste; indeed, we have 110 tried without success to prepare such emulsions with abrasives other than levigated alumina. Thus, in the case of finely powdered carborundum, we find that the abrasive in less than an hour separates from the 115 soap and water and settles to the bottom of the container, whereas with levigated alumina we have produced emulsions that stand without substantial separation for months at a time. We accordingly believe 120 125 130 135

that we are the first to utilize levigated alumina in a preparation of the character in question and the first to produce such a preparation in the form of a relatively permanent emulsion of abrasive, soap and water. By a relatively permanent emulsion we mean one that will stand for weeks at a time without substantial separation of the constituents.

10 The relative permanency of our emulsion is important because it obviates serious difficulties that would otherwise arise, both in the manufacture and the distribution and use of the strop dressing. That is to say, if the constituents were to separate materially in an hour or less, as in the case of carborundum above referred to, it would be very difficult to maintain a uniform composition during any commercially practical process of manufacturing the product and charging it into the containers. Furthermore, a rapid and easy separation of the constituents would result, while the product was on the shelf of the distributor or of the user, in the depositing and caking of the finely divided abrasive on the wall of the container so that it would be practically impossible to restore the emulsion by shaking. In the case of our improved strop dressing, when the constituents are properly proportioned, the emulsion mixture is so persistent that these difficulties are obviated.

15 While in the foregoing description we have set forth in detail the preferred

method of preparing our strop dressing and the preferred proportions of the ingredients, it should be understood that we do not intend to limit our invention in these respects except as defined in the appended 40 claims.

What we claim as our invention is:

1. An abrasive strop dressing consisting of a relatively permanent emulsion of levigated alumina, soap and water. 45

2. An abrasive strop dressing consisting of levigated alumina, soap and water in the following proportions by weight: levigated alumina thirty to fifty per cent., soap ten to twenty-five per cent., water thirty 50 to fifty-five per cent., the said substances being intimately mixed to form a paste.

3. An abrasive strop dressing consisting of levigated alumina, soap and water in substantially the following proportions by weight: levigated alumina forty-seven per cent., powdered soap twenty per cent., water thirty-three per cent., the said substances being intimately mixed to form a 55 paste.

We hereby assert that the above is a full and accurate description of our invention and in testimony whereof we have affixed our signatures in the presence of two witnesses.

L. G. WESSON.  
ZAY JEFFRIES.

Witnesses:

J. BURNS READ,  
THEODORE H. BARRETT.